

Patented Aug. 7, 1928.

1,679,479

# UNITED STATES PATENT OFFICE.

HANS LEEMANN, OF BOTTMINGERMUHLE-BINNINGEN, NEAR BASEL, AND GIOVANNI TAGLIANI, OF BASEL, SWITZERLAND, ASSIGNORS, BY MESNE ASSIGNMENTS, TO MUNITEX CORPORATION, OF LODI, NEW JERSEY, A CORPORATION OF NEW JERSEY.

## RESERVE DYEING ON VEGETABLE FIBERS.

No Drawing. Original application filed April 27, 1925, Serial No. 26,289, and in Germany May 7, 1924. Divided and this application filed May 20, 1926. Serial No. 110,539.

This application is divisional of application Ser. No. 26,289.

The hitherto known reserve processes consist of mechanical or chemical operations.

5 To the first type belongs the binding and covering of the vegetable fibers (yarns and fabrics) by substances insoluble in water so that the dyestuffs employed can only soak in and be fixed on the unbound or uncovered 10 parts of the fabric. To the second class belongs the application of certain agents, preferably of salts, which react chemically during the dyeing or during the development of the dyes. All these processes depend, 15 however, on certain conditions. If the reserve agents employed are removed during the dyeing process or during the development of the dyes, or if they do not resist these operations until the end of the dyeing, 20 then the desired reserve effect does not occur and the fabric is dyed uniformly throughout as if the reserving agents had not been used at all.

It is known from German specification No. 25 346,883 and others, that it is possible to render vegetable fibers (yarns, loose material, fabrics) completely immune against substantive dyestuffs by treating them after alkalization with solutions of aromatic 30 acid chlorides or aromatic sulpho acid chlorides. Both the alkalization and the action of the aromatic carboxylic acid or sulpho acid chlorides are so effected that the whole of the vegetable fibers is brought into 35 the solutions of the respective agents.

It has now been shown in a surprising manner that this esterification can also be used for the topical alteration of the vegetable fibers, in view of the production of reserve effects, for example in a suitable printing process. It was not at all to be foreseen from the more active treatment in solution that the short superficial and sparing local treatment, as it takes place for example in 40 the printing process, would suffice to produce the desired esterification. This process affords permanently reserving patterns with unexpected dyeing properties, which remain fast even after hot washing operations, after 45 hot neutral, acid or alkaline dye baths.

The production of such reserve effects is now utilized in the process for reserve dyeing on vegetable fibers forming the subject

of the present invention. This process consists in first treating topically the vegetable 55 fibers by a local printing with a suitable alkalizing agent, such for example as a concentrated alkaline solution, with or without thickening agent, with or without the addition of alcohol, with or without an alcoholic 60 solution of an alkali alcoholate, then in applying thereon in dry or moist condition, an esterifying aromatic acid chloride, such as an aromatic carboxylic acid chloride, or an aromatic sulpho acid chloride, in pure or 65 dissolved condition, and finally after the resulting esterification, in thoroughly washing the vegetable fibers being thus locally altered at the places of the aforesaid print, to constitute what is commonly termed as reserve 70 effects. Thereupon the thus topically altered fibers are dyed in one single bath with both a substantive and a convenient acid dyestuff. The substantive dyestuff is fixed by the unaltered parts, while the acid one 75 dyes the esterified parts of the fibers.

As dyestuffs, there may be used the usual coloring matters which are suitable for carrying out the improved process. The fibers may be in form of loose material, yarns or 80 fabrics.

### What we claim is:

1. A process for reserve dyeing on vegetable fabrics, which consist in treating topically the vegetable fibers by a local printing 85 with an alkalizing agent, thereupon applying an esterifying aromatic acid chloride to produce a topical alteration of the locally printed fiber, thus constituting reserve effects, then washing after the esterification, 90 and thereupon dyeing the thus topically altered fibers in one single bath with both a substantive and a convenient acid dyestuff.

2. A process for reserve dyeing on vegetable fibers, which consists in treating topically the vegetable fibers by a local printing with an alkalizing agent, thereupon applying an esterifying aromatic sulpho acid chloride to produce a topical alteration of the locally printed fiber, thus constituting 95 reserve effects, then washing after the esterification, and thereupon dyeing the thus topically altered fibers in one single bath with both a substantive and a convenient acid dyestuff.

3. A process for reserve dyeing on vege-

table fibers which comprises treating predetermined areas of said fibers with an alkalizing agent, esterifying said treated areas with an aromatic acid chloride whereby reserve effects are produced, washing said fibers and dyeing the thus treated areas in a bath containing both a substantive and an acid dyestuff.

4. A process for reserve dyeing on vegetable fibers which comprises treating predetermined areas of said fibers with an al-

kalizing agent, esterifying said treated areas with an aromatic sulpho acid chloride whereby reserve effects are produced, washing said fibers and dyeing the thus treated areas in a bath containing both a substantive and an acid dyestuff. 15

In witness whereof we have hereunto signed our names this 10th day of May, 1926.

HANS LEEMANN.  
GIOVANNI TAGLIANI.